



US007001653B2

(12) **United States Patent**  
Chen et al.

(10) **Patent No.:** US 7,001,653 B2  
(45) **Date of Patent:** Feb. 21, 2006

(54) **FUSING-STATION ROLLER**

(75) Inventors: **Jiann-Hsing Chen**, Fairport, NY (US); **Joseph A. Pavlisko**, Pittsford, NY (US); **Po-Jen Shih**, Webster, NY (US); **Robert A. Lancaster**, Hilton, NY (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **10/668,014**

(22) Filed: **Sep. 22, 2003**

(65) **Prior Publication Data**

US 2004/0121253 A1 Jun. 24, 2004

**Related U.S. Application Data**

(60) Provisional application No. 60/435,198, filed on Dec. 20, 2002.

(51) **Int. Cl.**

**B32B 1/08** (2006.01)  
**B32B 27/20** (2006.01)  
**B32B 27/30** (2006.01)  
**G03G 15/20** (2006.01)

(52) **U.S. Cl.** ..... **428/36.91**; 428/313.5; 428/332; 428/421; 399/333

(58) **Field of Classification Search** ..... 399/333; 492/56; 428/36.8, 36.91, 313.5, 315.9, 325, 428/328, 329, 332, 421, 422

See application file for complete search history.

(56) **References Cited****U.S. PATENT DOCUMENTS**

|             |         |                                   |
|-------------|---------|-----------------------------------|
| 3,615,972 A | 10/1971 | Morehouse, Jr. et al. .... 156/79 |
| 3,914,360 A | 10/1975 | Gunderman et al. .... 264/51      |
| 4,513,106 A | 4/1985  | Edgren et al. .... 521/58         |
| 4,984,027 A | 1/1991  | Derimiggio et al. .... 355/290    |

|              |         |                      |           |
|--------------|---------|----------------------|-----------|
| 5,292,606 A  | 3/1994  | Fitzgerald .....     | 428/35.8  |
| 5,336,539 A  | 8/1994  | Fitzgerald .....     | 428/36.8  |
| 5,450,183 A  | 9/1995  | O'Leary .....        | 355/285   |
| 5,464,698 A  | 11/1995 | Chen et al. ....     | 428/421   |
| 5,480,724 A  | 1/1996  | Fitzgerald .....     | 428/447   |
| 5,595,823 A  | 1/1997  | Chen et al. ....     | 428/421   |
| 5,654,052 A  | 8/1997  | Visser et al. ....   | 428/35.8  |
| 5,716,714 A  | 2/1998  | Chen et al. ....     | 428/473.5 |
| 5,754,931 A  | 5/1998  | Castelli et al. .... | 399/297   |
| 5,916,671 A  | 6/1999  | Dauber et al. ....   | 428/317.3 |
| 6,190,771 B1 | 2/2001  | Chen et al. ....     | 428/375   |
| 6,224,978 B1 | 5/2001  | Chen et al. ....     | 428/376   |
| 6,225,409 B1 | 5/2001  | Davis et al. ....    | 525/104   |
| 6,235,801 B1 | 5/2001  | Morales et al. ....  | 521/54    |

(Continued)

**OTHER PUBLICATIONS**

Cowie, Polymers: Chemistry and Physics of Modern Materials, 2<sup>nd</sup> Edition, pp. 8-10, 1991.\*

Hawley's Condensed Chemical Dictionary, 13th Edition, p. 995, Jan. 1999.

(Continued)

Primary Examiner—Ramsey Zacharia

(74) Attorney, Agent, or Firm—Carl F. Ruoff

(57) **ABSTRACT**

A controlled modulus fusing-station member inclusive of a durable, tough, elastically deformable layer incorporating hollow flexible filler particles. The elastically deformable layer is preferably a single layer on a substrate, the substrate preferably a core member of a fuser roller or a pressure roller. The elastically deformable layer is made from a dry formulation inclusive of: a fluoro-thermoplastic polymer powder; microspheres in the form of unexpanded microspheres or expanded microballoons; and solid filler particles including strength-enhancing filler particles and thermal-conductivity-enhancing filler particles. The dry formulation can be thermally cured or electron-beam cured. Preferably, the dry formulation is thermally cured and further includes a curing catalyst, preferably a peroxide catalyst. Alternatively, the curing catalyst can be a bisphenol residue.

**35 Claims, 2 Drawing Sheets**



U.S. PATENT DOCUMENTS

6,261,214 B1 7/2001 Meguriya ..... 492/56  
6,355,352 B1 3/2002 Chen et al. ..... 428/421  
6,361,829 B1 3/2002 Chen et al. ..... 427/380  
6,429,249 B1 8/2002 Chen et al. ..... 524/432  
6,486,441 B1 \* 11/2002 Chen et al. ..... 219/216  
6,490,430 B1 12/2002 Chen et al. ..... 399/333  
2002/0102410 A1 \* 8/2002 Gervasi et al. ..... 428/421

OTHER PUBLICATIONS

Office Action for copending Application No. 10/667,548, mailed Sep. 7, 2004.  
Office Action for copending Application No. 10/667,996, mailed Sep. 9, 2004.  
Office Action for copending Application No. 10/667,781, mailed Sep. 9, 2004.  
\* cited by examiner



FIG. 1



FIG. 2



FIG. 3

## 1

## FUSING-STATION ROLLER

## CROSS REFERENCE TO RELATED APPLICATION

Reference is made to and priority claimed from U.S. Provisional Application Ser. No. 60/435,198, filed Dec. 20, 2002, entitled IMPROVED FUSING-STATION ROLLER.

## FIELD OF THE INVENTION

The invention relates to electrostatography and to a fusing-station roller and method of making, and in particular to a deformable roller having a resilient layer made from a crosslinked thermoplastic fluorocarbon material incorporating both hollow fillers and solid fillers.

## BACKGROUND OF THE INVENTION

In electrostatographic imaging and recording processes such as electrophotographic printing, an electrostatic latent image is formed on a primary image-forming member such as a photoconductive surface and is developed with a thermoplastic toner powder to form a toner image. The toner image is thereafter transferred to a receiver member, e.g., a sheet of paper or plastic, and the toner image is subsequently fused or fixed to the receiver member in a fusing station using heat and/or pressure. The fusing station includes a heated fuser member which can be a roller, belt, or any surface having a suitable shape for fixing thermoplastic toner powder to the receiver member. Fusing typically involves passing the toned receiver member between a pair of engaged rollers that produce an area of pressure contact known as a fusing nip. In order to form the fusing nip, at least one of the rollers typically includes a compliant or deformable layer. Heat is transferred from a heated roller fuser member to the toner in the fusing nip, causing the toner to partially melt and attach to the receiver member.

Normally included in a compliant heated fuser member roller is a resilient or elastically deformable base cushion layer (e.g., an elastomeric layer). The base cushion layer is usually covered by one or more concentric layers, including a protective outer layer. The base cushion layer is typically bonded to a core member included in the roller, with the roller having a smooth outer surface. Where the fuser member is in the form of a belt, e.g., a flexible endless belt that passes around the heated roller, it commonly has a smooth outer surface which may also be hardened. Similarly, a resilient base cushion layer can be incorporated into a deformable pressure roller used in conjunction with a relatively hard fuser roller.

Simplex fusing stations attach toner to only one side of the receiver member at a time. In this type of station, the engaged roller that contacts the unfused toner is commonly known as the fuser roller and is a heated roller. The roller that contacts the other side of the receiver member is known as the pressure roller and is usually unheated. Either or both rollers can have a compliant layer on or near the surface. It is common for one of these rollers to be driven rotatably by an external source while the other roller is rotated frictionally by the nip engagement.

In a duplex fusing station, which is less common, two toner images are simultaneously attached, one to each side of a receiver passing through a fusing nip. In such a duplex fusing station there is no real distinction between fuser roller and pressure roller, both rollers performing similar functions, i.e., providing heat and pressure.

## 2

It is known that a compliant fuser roller, when used in conjunction with a harder or relatively non-deformable pressure roller, e.g., in a Digimaster 9110 machine made by Heidelberg Digital L.L.C., Rochester, N.Y., provides easy release of a receiver member from the fuser roller, because the distorted shape of the compliant surface in the nip tends to bend the receiver member towards the relatively non-deformable unheated pressure roller and away from the much more deformable fuser roller. On the other hand, when a conformable or compliant pressure roller is used to form the fusing nip against a hard fuser roller, such as in a Docutech 135 machine made by Xerox Corporation, Rochester, N.Y., a mechanical device such as a blade is typically necessary as an aid for releasing the receiver member from the fuser roller.

A conventional toner fuser roller includes a rigid cylindrical core member, typically metallic such as aluminum, coated with one or more synthetic layers usually formulated with polymeric materials made from elastomers. An elastically deformable or resilient base cushion layer, which may contain filler particles to improve mechanical strength and/or thermal conductivity, is typically formed on the surface of the core member, which core member may advantageously be coated with a primer to improve adhesion of the resilient layer. Roller cushion layers are commonly made of silicone rubbers or silicone polymers such as, for example, polydimethylsiloxane (PDMS) polymers disclosed, e.g., by the Chen, et al., patent (U.S. Pat. No. 6,224,978, assigned to Eastman Kodak Company, Rochester, N.Y.).

The most common type of fuser roller is internally heated, i.e., a source of heat is provided within the roller for fusing. Such a fuser roller generally has a hollow core member, inside of which is located a source of heat, usually a lamp. Surrounding the core member can be an elastomeric layer through which heat is conducted from the core member to the surface, and the elastomeric layer typically contains fillers for enhanced thermal conductivity [see for example the Fitzgerald patents (commonly assigned U.S. Pat. Nos. 5,292,606 and 5,336,539) and the Fitzgerald, et al., patent (commonly assigned U.S. Pat. No. 5,480,724)]. An internally heated fuser roller can be made using a condensation-polymerized silicone rubber material including solid filler particles, such as for example used in a NexPress 2100 digital color press (manufactured by NexPress Solutions LLC, Rochester, N.Y.).

Less common is an externally heated fuser roller, such as for example used in an Image Source 120 copier marketed by Eastman Kodak Company, Rochester, N.Y., which fuser roller is typically heated by surface contact with one or more heating rollers. An externally heated fuser roller can be made using an addition-polymerized silicone rubber material including solid filler particles. Externally heated fuser rollers are for example disclosed by the O'Leary patent (U.S. Pat. No. 5,450,183, assigned to Eastman Kodak Company, Rochester, N.Y.), the Derimiggio, et al., patent (commonly assigned U.S. Pat. No. 4,984,027), the Aslam, et al., patent application (U.S. patent application Ser. No. 09/680,134), and the Chen, et al., patent (commonly assigned U.S. Pat. No. 6,490,430). Inclusion of thermal-conductivity-enhancing fillers enhances heat transfer from one or more external heating rollers typically used for the external heating of the fuser roller. Moreover, the thermal-conductivity-enhancing fillers enable intermittent use of an auxiliary heating device located within the roller.

Some roller fusers rely on film splitting of a low viscosity oil to enable release of the toner and (hence) receiver member from the fuser roller. The release oil is typically

applied to the surface of the fuser from a donor roller coated with the oil provided from a supply sump. A donor roller is for example disclosed in the Chen, et al., patent (commonly assigned U.S. Pat. No. 6,190,771) which is hereby incorporated by reference.

Release oils (commonly referred to as fuser oils) are composed of, for example, polydimethylsiloxanes. When applied to the fuser roller surface to prevent the toner from adhering to the roller, fuser oils may, upon repeated use, interact with PDMS material included in the resilient layer(s) in the fuser roller, which in time can cause swelling, softening, and degradation of the roller. To prevent these deleterious effects caused by release oil, a thin barrier layer made of, for example, a cured fluoroelastomer and/or a silicone elastomer, is typically formed around the resilient cushion layer, as disclosed in the Davis, et al., patent (U.S. Pat. No. 6,225,409 assigned to Eastman Kodak Company, Rochester, N.Y.) and the Chen, et al., patents (U.S. Pat. No. 5,464,698, and 5,595,823, both assigned to Heidelberg Digital, L.L.C., Rochester, N.Y.). A fluoro-thermoplastic random copolymer outermost coating can also be used for this purpose, as disclosed in the Chen, et al., patents (commonly assigned U.S. Pat. Nos. 6,355,352 B1 and 6,361,829 B1). It is an object of the present invention to provide a fusing-station roller which does not require a coated barrier layer.

To rival the photographic quality produced using silver halide technology, it is desirable that electrostatographic multicolor toner images have high gloss. To this end, it is desirable to provide a very smooth fusing member contacting the toner particles in the fusing station. A gloss control outer layer (which also serves as a barrier layer for fuser oil) can be provided as disclosed in the Chen, et al., patent application (U.S. patent application Ser. No. 09/608,290). A fluorocarbon thermoplastic random copolymer useful for making a gloss control coating on a fuser roller is disclosed in the Chen, et al., patent (commonly assigned U.S. Pat. No. 6,429,249) which is hereby incorporated by reference.

In the fusing of the toner image to the receiver member, the area of contact of a conformable fuser roller with the toner-bearing surface of a receiver member sheet as it passes through the fusing nip is determined by the amount of pressure exerted by the pressure roller and by the characteristics of the resilient cushion layer. The extent of the contact area helps establish the length of time that any given portion of the toner image will be in contact with and heated by the fuser roller. It is generally advantageous to increase the contact time by increasing the contact area so as to result in a more efficient fusing process. However, unless the effective modulus for deforming a compliant roller in the nip is sufficiently low, high nip pressures are required to obtain a large nip area. Such high pressures can be disadvantageous and cause damage to a deformable roller, e.g., such as pressure set or other damage caused by edges of thick and/or hard receiver members as they enter or leave the nip. Hence a low modulus deformable roller is desirable.

It is known from the Chen, et al., patent (commonly assigned U.S. Pat. No. 5,716,714) that use of a relatively soft deformable fusing-station roller (e.g., a deformable pressure roller having a low effective modulus for deformation) can advantageously reduce the propensity of a fusing station nip to cause wrinkling of receiver members passing through the nip.

One way to try to create a low modulus fusing-station roller is to use a foamed material, e.g., a cured material having an open-cell or a closed-cell foam structure, with the material inclusive of suitable strength-enhancing and/or thermal-conductivity-enhancing fillers. Attempts to utilize

such foamed materials, for example as base cushion layers, have not generally been successful, for a number of reasons. The thermal conductivity of closed-cell structures tends to be disadvantageously low, even when squeezed in a fusing nip. Although an open-cell structure can be squeezed relatively flat in a fusing nip, the resilience typically becomes compromised because opposite walls within the foam tend to stick together under the heat and pressure of the nip. Moreover, foamed polymeric materials generally have poor tear strength, and shear strength also tends to be low. As a result, fusing-station rollers incorporating foamed base cushion layers are quite susceptible to damage and tend to age rapidly.

Suitable thermal conductivity of synthetic layers used in fusing-station rollers is attainable by the use of one or more suitable particulate fillers, the thermal conductivity being determined by the filler concentration. The thermal conductivity of most polymers is very low and the thermal conductivity generally increases as the concentration of thermally conductive filler particles is increased. However, if the filler concentration is too high, the mechanical properties of a polymer are usually compromised. For example, the stiffness of the synthetic layers may be increased by too much filler, e.g., so that there is insufficient compliance to create a wide enough nip for proper fusing. Moreover, too much filler will cause the synthetic layers to have a propensity to delaminate or crack, or otherwise cause failure of the roller. Because the mechanical requirements of fusing-station rollers require that the filler concentrations generally be moderate, the abilities of the layers to transport heat are thereby limited. In fact, the total concentration of strength-enhancing and thermal-conductivity-enhancing in prior art internally heated compliant fuser rollers has reached a practical maximum. As a result, the number of copies that can be fused per minute is limited, and this in turn can be the limiting factor in determining the maximum throughput rate achievable in an electrostatographic printer.

An auxiliary internal source of heat may optionally be used with an externally heated fuser roller, e.g., as disclosed in the Aslam, et al., patent (commonly assigned U.S. Pat. No. 6,567,641) and in the Chen, et al., patent (commonly assigned U.S. Pat. No. 6,490,430). Such an internal source of heat is known to be useful when the fusing station is quiescent and/or during startup when relatively cold toned receiver members first arrive at the fusing station for fusing therein. In order for such an auxiliary internal source of heat to be effective (when intermittently needed) the fuser roller must have a sufficiently large thermal conductivity. However, this requirement conflicts with a need to keep heat at the surface of an externally heated fuser roller, i.e., so as not to unnecessarily conduct heat into the interior which would compromise the fusing efficiency of the roller. On the other hand, it is important to have a high enough thermal conductivity at the surface of the fuser roller to ensure efficient transfer of heat to the fuser roller from one or more heating rollers contacting the surface. Moreover, in order to have high efficiency, externally heated fuser rollers rely to a certain extent on thermal conduction of heat around the surface of the roller.

Ways to improve upon the above-described limitations associated with externally heated elastically deformable fuser rollers (including an optional auxiliary internal source of heat) are disclosed in the Chen, et al., U.S. Patent Application and commonly assigned U.S. patent, Ser. No. 10/139,464 and U.S. Pat. No. 6,517,346, respectively). In Chen, et al., U.S. Pat. No. 6,517,346, an externally heated fuser roller having improved efficiency includes a core

member, a base cushion layer around the core member, a relatively thin heat storage layer around the base cushion layer, and an outer gloss control layer around the heat storage layer, wherein the heat storage layer is loaded with more thermally conductive filler than is the base cushion layer and hence has a higher thermal conductivity. In Chen, et al., U.S. patent application Ser. No. 10/139,464, a thin heat distribution layer is further included between the heat storage layer and the outer gloss control layer. While the fusing efficiencies relating to U.S. Pat. No. 6,517,346 and U.S. patent application Ser. No. 10/139,464 are much improved, the fuser rollers (respectively having 3-layer and 4-layer structures around the core member) are relatively expensive to manufacture, and may be susceptible to delamination with prolonged use.

It is known that instead of solid fillers, certain hollow fillers can be included in an addition-polymerized silicone rubber for the purpose of lowering rather than increasing the thermal conductivity of a deformable fuser roller, as disclosed in the Meguriya patent (U.S. Pat. No. 6,261,214, assigned to Shin-Etsu Chemical Company, Ltd., Tokyo, Japan). In particular, the Meguriya patent discloses incorporation into the silicone rubber of hollow filler particles (also known as microballoons) manufactured under the trademark EXPANCEL® available from Expance, (Sundsvall, Sweden and Duluth, Ga.).

Hollow microballoons are well known and are disclosed for example in the Morehouse, et al., patent (U.S. Pat. No. 3,615,972, assigned to Dow Chemical Company, Midland, Mich.). Microballoons are made from thermoplastic microspheres which encapsulate a liquid blowing agent, typically a hydrocarbon liquid. Such microspheres are made in unexpanded form. The walls of the unexpanded microspheres are generally impermeable to the liquid blowing agent, i.e., diffusion of molecules of the liquid blowing agent through the walls is typically negligible. An expanded form of a microsphere, i.e., a microballoon, is obtained by heating an unexpanded microsphere to a suitable temperature so as to vaporize the blowing agent, thereby causing the microsphere to grow to a much larger size. Too high of a heating temperature can result in some loss of internal vapor pressure and a shrinking of the microballoon. Methods for expanding microspheres are disclosed in numerous patents, such as, for example the Gunderman, et al., patent (U.S. Pat. No. 3,914,360, assigned to Dow Chemical Company, Midland, Mich.), the Edgren, et al., patent (U.S. Pat. No. 4,513,106, assigned to KemaNord AB, Stockholm, Sweden) and the Morales, et al., patent (U.S. Pat. No. 6,235,801 B1). Expansion is generally irreversible after cooling, and the expanded microballoon form is stable under normal ambient conditions and can be sold as a dry powder or alternatively as a slurry in a liquid vehicle. Expanded microspheres or microballoons which are available commercially can be incorporated into various materials, such as, for example, to make improved paints or lightweight parts. Unexpanded microspheres are also available commercially for incorporation into various types of materials (e.g., expandable inks) or for manufacture of solid parts, e.g., by thermal curing in a mold so as to expand the microspheres. The shell material of certain microsphere particles can include finely divided inorganic particles, e.g., silica particles.

The use of microspheres in a compressible layer of a digital printing blanket carcass is disclosed in the Castelli, et al., patent (U.S. Pat. No. 5,754,931, assigned to Reeves Brothers, Inc., Spartanburg, S.C.). The microspheres are uniformly distributed in a matrix material which includes thermoplastic or thermosetting resins.

The Dauber, et al., patent (U.S. Pat. No. 5,916,671, assigned to W. L. Gore & Associates, Inc., Newark, Del.) discloses a resilient gasket made of a composite of polytetrafluoroethylene and resilient expandable microspheres.

There remains a need to provide for an electrostatographic machine, an improved fusing station having high productivity which includes fusing-station members that are simple in construction, are very durable, and are made of material that can resist gouges or pressure damage from edges of receiver members moving through a high pressure fusing nip.

Specifically, there remains a need for a tough, long lasting fuser roller which has preferably only one layer coated on a core member, and which is thereby simple in structure by comparison with multi-layer prior art fuser rollers. This single layer is required to be chemically unreactive, stable at high temperatures, and impervious to fuser oil. Moreover, there remains a need for an improved pressure roller having a similarly simple single-layer structure and which has similar properties.

A fluoro-thermoplastic polymer crosslinked by curing is a desirable material for making fuser rollers and pressure rollers, because of low surface energy, chemical inertness, imperviousness to fuser oil, and high-temperature stability. It is an object of the invention to provide a fusing-station roller inclusive of an elastically deformable crosslinked fluoropolymer layer made from a fluoro-thermoplastic formulation.

## SUMMARY OF THE INVENTION

The invention provides an improved fusing-station member for use in a fusing station of an electrostatographic machine, the fusing-station member including an elastically deformable synthetic fluoropolymer layer incorporating flexible hollow filler particles. The fusing-station member includes a fuser roller and a pressure roller. The fusing station has a fusing nip wherein a toner image is fixed to a receiver member being moved through the fusing nip. The improved fusing-station member is simple in construction, long lasting, highly durable, and has just one synthetic layer.

In certain embodiments, the fusing-station member is an internally heated or externally heated fuser roller forming a fusing nip with a compliant, relatively soft, pressure roller. The fuser roller includes a core member and an elastically deformable layer formed around the core member. The elastically deformable layer is a highly crosslinked fluoropolymer material made by curing at an elevated temperature an uncured formulation which includes a fluoro-thermoplastic polymer compounded with three types of filler particles, namely hollow flexible microballoon particles, strength-enhancing solid particles, and thermal-conductivity-enhancing solid particles. A weight percent of fluorine in the formula weight of the fluoro-thermoplastic polymer preferably has a lower limit of about 70%.

In alternative fuser roller embodiments, unexpanded microspheres in lieu of the hollow flexible microballoon particles are compounded with strength-enhancing solid filler particles and thermal-conductivity-enhancing solid filler particles in an uncured fluoro-thermoplastic formulation for making the elastically deformable layer.

In other embodiments, the fusing-station member is a pressure roller forming a fusing nip with a compliant relatively soft fuser roller. The pressure roller includes a core member and an elastically deformable layer formed around the core member. The elastically deformable layer is a highly crosslinked fluoropolymer material made by curing at

elevated temperatures an uncured formulation which includes a fluoro-thermoplastic polymer compounded with three types of filler particles, namely hollow flexible microballoon particles, strength-enhancing solid particles, and thermal-conductivity-enhancing solid particles. A weight percent of fluorine in the formula weight of the fluoro-thermoplastic polymer preferably has a lower limit of about 70%.

In alternative pressure roller embodiments, unexpanded microspheres in lieu of the hollow flexible microballoon particles are compounded with strength-enhancing solid filler particles and thermal-conductivity-enhancing solid filler particles in an uncured fluoro-thermoplastic formulation for making the elastically deformable layer.

The invention, and its objects and advantages, will become more apparent in the detailed description of the preferred embodiment presented below.

#### BRIEF DESCRIPTION OF THE DRAWINGS

In the detailed description of the preferred embodiments of the invention presented below, reference is made to the accompanying drawings in which the relative relationships of the various components are illustrated. For clarity of understanding of the drawings, relative proportions depicted or indicated of the included elements may not be representative of the actual proportions, and some of the dimensions may be selectively exaggerated.

FIG. 1 shows a cross-sectional view of a fusing-station roller in the form of a fuser roller of the invention;

FIG. 2 shows a cross-sectional view of a fusing-station roller in the form of a pressure roller of the invention; and

FIG. 3 schematically illustrates exemplary steps for making a fuser roller as shown in FIG. 1 and a pressure roller as shown in FIG. 2.

#### DETAILED DESCRIPTION OF THE PREFERRED EMBODIMENTS

Fusing stations and fusing-station rollers for use according to this invention are readily includable in typical electrostatographic reproduction or printing machines of many types, such as for example electrophotographic color printers.

The invention relates to an electrostatographic machine for forming a toner image on a receiver member and utilizing a fusing station for thermally fusing or fixing the unfused toner image to the receiver member, e.g., paper or a plastic sheet. The fusing station, which includes a heated fuser member forming a fusing nip with a pressure member, applies heat and pressure to fix the unfused toner image carried on the receiver member as the receiver member is moved through the fusing nip. The fuser member has an elastically deformable surface, and the pressure member is a relatively softer, compliant, member. The fuser member can be a roller, belt, or any surface suitable for fixing thermoplastic toner powder to the receiver member. A fuser member and a pressure member are referred to herein as fusing-station members, e.g., fusing-station rollers.

A fusing-station roller of the invention is a controlled-modulus roller preferably made from a cured fluoro-thermoplastic polymer. A preferred fluoro-thermoplastic polymer is disclosed in the Chen, et al., patent (commonly assigned U.S. Pat. No. 6,429,249). Fluoro-thermoplastic polymers are commercially available, such as for example fluorocarbon thermoplastic random copolymers known as THV materials sold by 3M® Corporation, St. Paul, Minn.,

e.g., THV 200. In preferred fusing-station embodiments, the fluoro-thermoplastic material is cured to form a resilient crosslinked fluoropolymer material. Hitherto, because of a high stiffness due in part to included solid filler particles, crosslinked fluoro-thermoplastic polymeric materials have not been useful for making deformable layers of fusing-station rollers. An important feature of the crosslinked fluoropolymer material used in the invention is that the material incorporates both solid and hollow filler particles. Inclusion of the hollow filler particles according to the invention provides the requisite resilience to make such fusing-station rollers practical.

In certain embodiments, the fusing-station roller is an externally heated fuser roller for use with a relatively soft pressure roller, which fuser roller preferably includes an auxiliary internal heat source. In alternative embodiments, the fuser roller is preferably internally heated. In other embodiments, the fusing-station roller is a resilient pressure roller for use with a relatively soft, compliant, fuser roller, which compliant fuser roller can be externally heated or internally heated as may be suitable.

The fusing station preferably includes the fuser roller and the pressure roller in frictional driving relation. Typically, one of the rollers is rotated via a motor, and the other roller is frictionally rotated by engagement in the fusing nip, wherein the fuser roller comes into direct contact with the unfused toner image as the receiver member is moved through the nip. An externally heated fuser roller is preferably directly heated by a dedicated external source of heat, such as by contact with one or more external heating rollers, in a well known manner. Alternatively, an externally heated fuser roller may be heated via absorbed radiation, e.g., as provided by one or more lamps, or by any other suitable external source of heat. An internally heated fuser roller includes an internal heat source, such as a lamp, as is well known. The pressure roller, which preferably is not directly heated, is typically indirectly heated to a certain extent via contact in the fusing nip.

Preferably, an oiling mechanism is provided for applying a fuser oil or release oil to the surface of the fuser roller, as is well known. For example, the oiling mechanism can be a donor roll mechanism for applying a silicone oil, e.g., from a sump included in the donor roll mechanism. The fuser oil thus applied by the oiling mechanism serves to release a receiver member carrying a fused image from the fuser roller after passage of the receiver member through the fusing nip. The fuser oil is also used for the purpose of preventing offset, whereby melted toner material can be disadvantageously deposited on the fuser roller. A preferred fuser oil is sold as No. 8707 oil by Walker Silicone, which oil is an amine-functionalized polydimethylsiloxane oil having a viscosity of about 300 centipoise.

In prior art, conformable layers of fusing-station rollers are typically protected by a coated outer barrier layer or protective layer so as to prevent harmful effects caused by interaction with hot fuser oil molecules. An advantageous feature of the preferred embodiment of the invention is that no such outer layer is needed.

It is preferred for a cleaning station of the known type to be provided for cleaning the surface of the fuser roller. Additionally or alternatively, a cleaning station can be provided for cleaning the surface of the pressure roller.

The toner image in an unfused state may include a single-color toner or it may include a composite image of at least two single-color toner images, e.g., a composite image in full color made, for example, from superimposed black, cyan, magenta, and yellow single-color toner images. The

## 9

unfused toner image is previously transferred, e.g., electrostatically, to the receiver member from one or more toner image bearing members such as primary image-forming members or intermediate transfer members. It is well established that for high quality electrostatographic color imaging with dry toners, small toner particles are necessary.

Fusing-station rollers of the invention are suitable for the fusing of dry toner particles having a mean volume weighted diameter in a range of approximately between 2  $\mu\text{m}$ –9  $\mu\text{m}$ , and more typically, about 7  $\mu\text{m}$ –9  $\mu\text{m}$ , but the invention is not restricted to these size ranges. The fusing temperature to fuse such particles included in a toner image on a receiver member is typically in a range of 100° C.–200° C., and more usually, 140° C.–180° C., but the invention is not restricted to these temperature ranges.

The electrostatographic reproduction or printing may utilize a photoconductive electrophotographic primary image-forming member or a non-photoconductive electrographic primary image-forming member. Particulate dry or liquid toners may be used.

Turning now to FIG. 1, a cross-sectional view of a fusing-station member is illustrated in the form of a fuser roller embodiment of the invention, identified by the numeral 10. Fuser roller 10 is an elastically deformable roller preferably for use with a relatively soft pressure roller. Fuser roller 10 includes a substrate in the form of a core member 16 and a resilient layer 14 formed on the core member. Optionally, fuser roller 10 further can include a protective layer or gloss control layer 12 coated on the resilient layer. As described in detail below, an important feature of the fuser roller 10 is the presence of flexible hollow filler particles 18 incorporated in resilient layer 14.

The core member 16 is preferably rigid and preferably made of a thermally conductive material such as a metal, preferably aluminum, and has a cylindrical outer surface. The core member is typically (but not necessarily) generally tubular, as shown. The resilient layer 14 is preferably formed on the core member 16 by using an extrusion and curing technique, followed by successive post-coating curings and grindings as may be necessary.

Fuser roller 10, when being utilized in a fusing station, forms a fusing nip with a preferably relatively soft pressure roller in well known fashion (pressure roller and fusing nip not illustrated in FIG. 1). It is important to have a contact width in the fusing nip which is large so as to effect efficient transfer of heat from fuser roller 10 to a toner image carried on a receiver member moved through the nip. A preferred contact width in the fusing nip (measured perpendicular to the fuser roller rotational axis) is in a range of approximately between 13 mm–22 mm.

Resilient layer (RL) 14 is a highly crosslinked fluoropolymer made by a curing of an uncured formulation which includes a fluoro-thermoplastic polymer. RL 14 preferably includes three types of filler particles, namely, flexible hollow filler particles, strength-enhancing solid particles, and thermal-conductivity-enhancing solid particles. RL 14 is an elastically deformable layer; hereinafter “elastically deformable” is defined as pertaining to a Shore A durometer less than about 80.

Certain preferred embodiments of RL 14 are made by curing of formulations which include the hollow filler particles as pre-expanded hollow microballoons commercially available as manufactured powders, which pre-expanded hollow microballoons are made from unexpanded microspheres via a thermal expansion process (see Morehouse, et al., U.S. Pat. No. 3,615,972, assigned to Dow Chemical Company, Midland, Mich.). For these embodiments, the

## 10

uncured formulations preferably exclude unexpanded microspheres. Expanded microballoon powders for use in the invention are obtainable from Expance (Sundsvall, Sweden and Duluth, Ga.). Expance is a part of the business unit, Casco Products, within Akzo Nobel, in the Netherlands. The flexible microballoons can have any suitable diameter(s). It is preferred that the included microballoons have diameters of up to approximately 120  $\mu\text{m}$ .

Flexible microballoon particles included in an uncured formulation for making RL 14 can have any suitable diameter(s). It is preferred that the included microballoons have diameters of up to approximately 120  $\mu\text{m}$ .

Alternative preferred embodiments of RL 14 incorporating the hollow filler particles are made by thermal curing of alternative formulations which include unexpanded microspheres. The hollow filler particles in these alternative embodiments are formed from the unexpanded microspheres by thermal expansion into microballoons during the curing process at elevated temperatures. Preferably, such alternative uncured formulations (which also include strength-enhancing and thermal-conductivity-enhancing solid particles) exclude expanded microballoons. Varieties of such unexpanded microspheres are available commercially for subsequent thermal expansion during the curing process, which varieties can produce different ranges of expanded sizes after such heating. Unexpanded microspheres for use in uncured formulations are commercially obtainable from Expance (Sundsvall, Sweden and Duluth, Ga.). A wide variety of post-curing size distributions of expanded microballoons having at least one distinguishable size can be created in the alternative embodiments of RL 14 by using one or more varieties of unexpanded microspheres in the uncured alternative resilient layer formulation.

Elevated temperatures useful for thermally curing RL 14 preferably exceed 150° C., as described below.

A relatively narrow size distribution of microballoon particles (in pre-expanded form) can be used to make RL 14. Alternatively, a bimodal distribution or a broad size distribution of microballoon particles can be used. A bimodal distribution can for example be made by incorporating two relatively narrow size distributions of expanded microballoons into the uncured formulation. Various sizes of expanded microballoons are commercially available, so that a wide variety of tailored size distributions can be assembled and employed in uncured formulations for making RL 14.

The walls of microspheres that can be used in uncured formulations for making RL 14, i.e., microspheres having a form that includes at least one of an expanded microballoon form and an unexpanded microsphere form, are preferably made from a polymeric material polymerized as a homopolymer or as a copolymer from one or more of the following group of monomers: acrylonitrile, methacrylonitrile, acrylate, methacrylate, and vinylidene chloride. However, any suitable monomer may be used.

The walls of expanded microsphere particles or of unexpanded microspheres useful for making RL 14 can include finely divided solid particles. Inorganic particles, e.g., oxide particles, or any other suitable finely divided inorganic particles, can be included in the walls. Additionally or alternatively, the walls of unexpanded or expanded microspheres may include finely divided organic polymeric particles.

Hereinafter the term “microsphere” refers to both unexpanded or expanded particles useful in uncured formulations for making RL 14, and the term “microballoon” generally refers to expanded microspheres. A concentration in an uncured formulation of either unexpanded or expanded

## 11

microsphere particles is referred to as a microsphere concentration. Predetermined microsphere concentrations in an uncured formulation for making RL 14 are preferably in a range of approximately between 0.25%–10% by weight (w/w), and more preferably, 0.5%–4% (w/w).

Any suitable volume percentage of microspheres may be used in an uncured formulation for making RL 14. Moreover, at least one distinguishable size of expanded microballoons (or alternatively unexpanded microspheres) can be used, having either one mean size or a combination of sizes. If expanded balloon microspheres are used, the volume percentage in the uncured formulation can be large, preferably in a range of approximately between 30%–90% by volume (v/v).

A preferred concentration by weight of strength-enhancing solid particles (sometimes referred to as structural fillers) in an uncured formulation for making RL 14 is in a range of approximately between 2.5%–10% (w/w). Any suitable volume percentage of strength-enhancing solid particles may be used in the uncured formulation for making RL 14.

A preferred concentration by weight of thermal-conductivity-enhancing solid particles in an uncured organosiloxane formulation for making RL 14 is in a range of approximately between 40%–70% (w/w). Any suitable volume percentage of thermal-conductivity-enhancing solid particles may be used in the uncured formulation for making RL 14.

Strength-enhancing solid filler particles are preferably silica particles, e.g., mineral silica particles or fumed silica particles. Other strength-enhancing solid fillers which can be included are particles of zirconium oxide, boron nitride, silicon carbide, carbon black, and tungsten carbide. The strength-enhancing particles preferably have a mean diameter in a range of approximately between 0.1  $\mu\text{m}$ –100  $\mu\text{m}$ , and more preferably, a mean diameter between 0.5  $\mu\text{m}$ –40  $\mu\text{m}$ .

Preferred thermal-conductivity-enhancing solid filler particles include particles of aluminum oxide, iron oxide, copper oxide, calcium oxide, magnesium oxide, nickel oxide, tin oxide, zinc oxide, graphite, carbon black, or mixtures thereof. The thermal-conductivity-enhancing particles preferably have a mean diameter in a range of approximately between 0.1  $\mu\text{m}$ –100  $\mu\text{m}$ , and more preferably, a mean diameter between 0.5  $\mu\text{m}$ –40  $\mu\text{m}$ . In a preferred embodiment, RL 14 includes aluminum oxide thermal-conductivity-enhancing particles.

For internally heated embodiments of fuser roller 10, the resilient layer 14 preferably has a thermal conductivity in a range of approximately between 0.08 BTU/hr/ft $^{\circ}$  F.–0.7 BTU/hr/ft $^{\circ}$  F., and more preferably, in a range of approximately between 0.2 BTU/hr/ft $^{\circ}$  F.–0.5 BTU/hr/ft $^{\circ}$  F.

For externally heated embodiments of fuser roller 10, the thermal conductivity of resilient layer 14 preferably has an upper limit of approximately 0.4 BTU/hr/ft $^{\circ}$  F. More preferably, the thermal conductivity of RL 14 in a range of approximately between 0.1 BTU/hr/ft $^{\circ}$  F.–0.35 BTU/hr/ft $^{\circ}$  F.

Resilient layer 14 preferably has a Shore A durometer in a range of approximately between 50–80, and more preferably, in a range of approximately between 60–70.

A thickness of resilient layer 14 preferably has an upper limit of approximately 0.1 inch. More preferably, the thickness of resilient layer 14 is in a range of approximately between 0.005 inch–0.02 inch.

A preferred fluoro-thermoplastic polymer for making resilient layer 14 is a random copolymer of the monomers vinylidene fluoride ( $\text{CH}_2=\text{CF}_2$ ), hexafluoropropylene

## 12

( $\text{CF}_2=\text{CF}(\text{CF}_3)$ ), and tetrafluoroethylene ( $\text{CF}_2=\text{CF}_2$ ), the random copolymer having a composition of:



wherein,

x is from 1 to 50 mole percent,

y is from 9 to 59 mole percent,

z is from 40 to 90 mole percent,

x+y+z equals 100 mole percent.

A weight percent of fluorine in the formula weight of the fluoro-thermoplastic polymer for making resilient layer 14 has a lower limit of about 70%.

A molecular weight of the fluoro-thermoplastic polymer for making resilient layer 14 is in a range of approximately between 50,000–800,000, and more preferably, in a range of approximately between 80,000–200,000.

As an alternative to fuser roller 10, the fuser member can be in the form of a flexible web (not illustrated). This web is heated for fusing in any suitable way. For example, the web can be pressed against the pressure roller by a heated back-up roller in the fusing station, such that a receiver member is moved between the web and the pressure roller for fixing a toner image thereto. The web preferably includes an elastically deformable or resilient layer formed on any suitable substrate, wherein the resilient layer includes flexible hollow filler particles and has a composition preferably similar to that of resilient layer 14. Thus the resilient layer is made with a formulation including microsphere particles (i.e., having a form that includes at least one of an expanded microballoon form and an unexpanded microsphere form) and suitable solid fillers, such as thermal-conductivity-enhancing solid filler particles and strength-enhancing solid filler particles.

A preferred relatively soft pressure roller (not illustrated) for use with fuser roller 10 includes a core member with a compliant base cushion layer preferably formed on the core member and a topcoat layer on the base cushion layer. The core member of the relatively soft pressure roller is preferably an aluminum cylinder. The thermal conductivity of the base cushion layer, while not critical, is preferred to be small enough so as not to drain a critical amount of heat from the fusing nip. A preferred base cushion layer of the relatively soft pressure roller is made of any elastomeric material for use at elevated temperatures, such as, for example, a highly crosslinked polydimethylsiloxane elastomer. The base cushion layer preferably includes a particulate filler. The topcoat layer, preferably having a thickness in a range of approximately between 0.001 inch–0.004 inch, is preferably made of a fluoropolymer, such as, for example, the fluorocarbon thermoplastic random copolymer of vinylidene fluoride, tetrafluoroethylene and hexafluoropropylene disclosed in the Chen, et al., patents (commonly assigned U.S. Pat. Nos. 6,355,352 B1 and 6,429,249). A preferred soft pressure roller can be similar to pressure rollers included in a NexPress 2100 digital color press (manufactured by NexPress Solutions LLC, Rochester, N.Y.).

A fusing station including the above-described relatively hard fuser roller 10 and a relatively soft compliant pressure roller advantageously provides a robust fusing mechanism. In particular, the cured fluoro-thermoplastic resilient layer 14 incorporating hollow microballoons is very tough and durable, thereby providing a long-lasting roller. Resilient layer 14 is resistant to gouging or scratching and also resistant to high-pressure damage from the edges of receiver members passing through the fusing station. In addition to

these advantages, fuser roller **10** has a very simple construction, i.e., a single layer formed on the core member **16**.

Turning now to FIG. 2, a cross-sectional view of a fusing-station member is illustrated in the form of a pressure roller embodiment of the invention, identified by the numeral **20**. Pressure roller **20** is preferably for use with a relatively soft, compliant, fuser roller. The pressure roller **20** includes a substrate in the form of a core member **26** and a resilient layer **24** formed on the core member. Optionally, pressure roller **20** further can include a protective layer or gloss control layer **22** coated on the resilient layer. In pressure roller **20** are flexible hollow filler particles **28** that are incorporated in resilient layer **24**. The core member **26** is similar to core member **16** of fuser roller **10**.

The resilient layer **24** of pressure roller **20** is preferably made from a highly crosslinked fluoro-thermoplastic material, and is similar in all respects to resilient layer **14** of fuser roller **10**. Thus RL **24** is made by curing a fluoro-thermoplastic formulation which preferably includes three types of filler particles, namely: strength-enhancing solid particles, thermal-conductivity-enhancing solid particles, and microsphere particles in unexpanded or expanded microballoon form. The microspheres used for RL **24** are preferably similar to those used for RL **14**, i.e., preferably made from a polymeric material polymerized as a homopolymer or as a copolymer from one or more of the following group of monomers: acrylonitrile, methacrylonitrile, acrylate, methacrylate, and vinylidene chloride. Also, the walls of the expanded microballoon particles or unexpanded microspheres can include finely divided inorganic particles, e.g., oxide particles, or any other suitable finely divided inorganic particles, preferably silica particles. Additionally or alternatively, the microsphere walls may include finely divided organic polymeric particles.

Certain preferred embodiments of RL **24** are made by inclusion of expanded microballoons in the uncured formulations, in a similar manner as for making RL **14** of fuser roller **10** (i.e., with unexpanded microspheres preferably excluded). Various sizes of microballoon particles can be used as may be suitable.

For making alternative preferred embodiments of RL **24** of pressure roller **20**, the corresponding alternative uncured formulations include unexpanded microspheres (i.e., with expanded microballoons preferably excluded). A wide variety of tailored size distributions can be assembled and employed in these alternative uncured formulations.

Predetermined microsphere concentrations in an uncured formulation for making RL **24** are preferably in a range of approximately between 0.25%–10% by weight (w/w), and more preferably, 0.5%–4% (w/w).

Any suitable volume percentage of microspheres may be used in the uncured formulation for RL **24**. Moreover, any suitable sizes of expanded microballoons (or alternatively unexpanded microspheres) can be used, having either one mean size or a combination of sizes. If expanded balloon microspheres are used, the volume percentage in the uncured formulation can be large, typically in a range of approximately between 30%–90% by volume (v/v).

A preferred concentration by weight of strength-enhancing solid particles (sometimes referred to as structural fillers) in an uncured formulation for making RL **24** is in a range of approximately between 2.5%–10% (w/w). Any suitable volume percentage of strength-enhancing solid particles may be used in the uncured organosiloxane formulation for making RL **24**.

A preferred concentration by weight of thermal-conductivity-enhancing solid particles in an uncured formulation

for making RL **24** is in a range of approximately between 40%–70% (w/w). Any suitable volume percentage of thermal-conductivity-enhancing solid particles may be used in the uncured formulation for making RL **24**.

In an alternative embodiment to pressure roller **20**, solid filler particles having primarily a strength-enhancing property are included in an uncured formulation for making RL **24**, and solid filler particles having primarily a thermal-conductivity-enhancing property are omitted.

Preferred for RL **24** are strength-enhancing solid filler particles and thermal-conductivity-enhancing solid filler particles of similar types and having similar sizes as preferably used for RL **14** of fuser roller **10**.

The resilient layer **24** preferably has a thermal conductivity in a range of approximately between 0.1 BTU/hr/ft<sup>2</sup>/F–0.2 BTU/hr/ft<sup>2</sup>/F.

Resilient layer **24** preferably has a Shore A durometer in a range of approximately between 50–80, and more preferably, approximately between 60–70.

A thickness of resilient layer **24** preferably has an upper limit of approximately 0.1 inch. More preferably, the thickness of resilient layer **24** is in a range of approximately between 0.005 inch–0.02 inch.

A preferred relatively soft fuser roller for use with pressure roller **20** includes a core member with a base cushion layer preferably formed on the core member and a topcoat layer on the resilient layer. The core member of the relatively soft fuser roller is preferably an aluminum cylinder. The base cushion layer preferably includes thermal-conductivity-enhancing and strength-enhancing particulate fillers. The base cushion layer can for example, be made of a crosslinked polydimethylsiloxane elastomer. The topcoat layer, preferably having a thickness in a range of approximately between 0.0015 inch–0.0040 inch, is preferably made of a fluoropolymer, such as for example the fluorocarbon thermoplastic random copolymer material made from copolymerized vinylidene fluoride, tetrafluoroethylene and hexafluoropropylene disclosed in the Chen, et al., patents (commonly assigned U.S. Pat. Nos. 6,355,352 B1 and 6,429,249). The relatively soft fuser roller can be heated for fusing in any known manner, e.g., using an internal heat source and/or an external heat source.

A fusing station including the above-described relatively hard pressure roller embodiment **20** and a relatively soft compliant fuser roller advantageously provides a robust fusing mechanism. In particular, a cured fluoro-thermoplastic resilient layer **24** incorporating hollow microballoons is very tough and durable, thereby providing a long-lasting roller. Resilient layer **24** is resistant to gouging or scratching and also resistant to high-pressure damage from the edges of receiver members passing through the fusing station. In addition to these advantages, pressure roller **20** can have a very simple construction, i.e., a single layer formed on the core member **26**.

Forming the resilient layer on a core member so as to make a fusing-station roller of the invention is now described in general terms, with reference to FIG. 3. An uncured formulation is first prepared, e.g., for making layer **14** or **24** of fuser rollers **10** and **20**. A respective uncured formulation includes ingredients as dry powders which are mixed together by any suitable means, e.g., manually or via a mechanical mixing device. Thus to prepare an uncured formulation, the microsphere particles and the strength-enhancing and thermal-conductivity-enhancing filler particles are combined with fluoro-thermoplastic polymer particles and blended into a uniform mixture, which mixture further includes as may be necessary a curing catalyst or a

## 15

curing agent. The fluoro-thermoplastic particles preferably have diameters in a range of approximately between 0.01 mm–1 mm. The microsphere particles can be pre-expanded microballoons, or they can be unexpanded microspheres which are transformed into microballoons during a thermal curing process. Pre-expanded microballoons can for example be flexible hollow DE 092 particles approximately 120  $\mu\text{m}$  in diameter (available from ExpanceL, Duluth, Ga.). The DE 092 particles have walls made of a copolymer of polyacrylonitrile and polymethacrylonitrile, the walls incorporating 3%–8% (w/w) finely divided silica.

FIG. 3 includes a simplified drawing representing an extrusion process for forming a resilient layer on a core member of a fusing-station roller. An extrusion apparatus 150 includes a die 130 through which an uncured formulation 125 is extruded in direction of arrows A, A' so as to produce a tubular covering around a core member 100. During extrusion, the uncured formulation 125 is heated to a temperature above the melting point of the fluoro-thermoplastic polymer included in the uncured formulation. This temperature is generally too low to effect a curing of the uncured formulation 125. For a preferred fluoro-thermoplastic polymer such as for example THV 200, the extrusion temperature is in a range of approximately between 80° C.–200° C., and more preferably, between 160° C.–180° C. An uncovered core member 100 is initially at a suitable temperature, which suitable temperature is preferably maintained during the extrusion process until the tubular covering is complete. A mechanism (not illustrated) is provided for appropriately cutting the extruded material so that the core member 100 plus completed covering can be removed from the extrusion apparatus 150.

At least three different ways of curing are contemplated by the invention, as indicated in the right hand portion of FIG. 3.

A first way, indicated by arrow "a", is a peroxide-catalyzed thermal curing process. A precursor roller 140 (formed in extrusion apparatus 150 and which includes core member 100 and an uncured layer 125) is cured at an elevated temperature, the uncured layer 125 including a thermally activated peroxide catalyst. The microsphere particles incorporated into uncured layer 125 can be in the form of expanded microballoons, or alternatively they can be unexpanded microspheres which are transformed into microballoons during the thermal curing process. The peroxide-catalyzed curing is carried out for a preferred time of approximately 1 hour at a preferred temperature in a range of approximately between 150° C.–200° C. However, any suitable curing time can be used. A preferred peroxide catalyst is 2,5 dimethyl-2, 5 di(t-butylperoxy)-hexane, obtainable under the registered trademark LUPERCO® 101 from Lucidol Division of Pennwalt Corporation, Buffalo, N.Y. The LUPERCO® 101 is used at a concentration of about 3 pph by weight in the uncured formulation. This catalyst requires a co-agent, which co-agent is also included in the uncured formulation, the co-agent preferably trially cyanurate, obtainable under the trade name TAC from American Cyanamid, Wayne, N.J. The TAC co-agent is incorporated at a concentration of about 3 pph by weight in the uncured formulation.

A second way of curing a prototype roller, indicated by arrow "b", is a bisphenol thermal curing process. A precursor roller 140' (formed in extrusion apparatus 150 and including core member 100 and an uncured layer 125') is cured at an elevated temperature, the uncured layer 125' incorporating a curing agent preferably including benzyl triphenyl phosphonium chloride. The microsphere particles

## 16

incorporated into uncured layer 125" can be in the form of expanded microballoons, or alternatively they can be unexpanded microspheres which are transformed into microballoons during the thermal curing process. Preferably the microsphere particles are unexpanded microspheres. The bisphenol thermal curing is carried out for a preferred time of up to approximately 1 hour at a preferred temperature in a range of approximately between 250° C.–300° C. However, any suitable curing time can be used. A preferred commercial curing agent is obtainable under the trade name Curative 50 (a bisphenol residue) from E. I. Dupont and Nemours. The Curative 50 is used at a concentration of about 3 pph by weight in the uncured formulation.

It is known that at high temperatures microballoons have a propensity to shrink. Therefore the peroxide catalyzed thermal curing process is generally preferred over the bisphenol curing process because the curing temperature is significantly lower.

A third way of curing a prototype roller, indicated by arrow "c", is via electron beam process (e-beam curing). A precursor roller 140" (formed in extrusion apparatus 150 and including core member 100 and an uncured layer 125") is cured by exposure to a high power electron beam in well known fashion. Thus the e-beam curing can be carried out by rotating the precursor roller 140" around its longitudinal axis so that the surface moves past either a rastered or a fixed source of electrons. No curing catalyst nor curing agent is used for the e-beam curing, which is advantageous. However, owing to the limited penetration of electron beams, e-beam curing is preferred for making relatively thin resilient layers, preferably thinner than about 0.02 inch. The microsphere particles incorporated into uncured layer 125" are preferably in the form of expanded microballoons.

Although e-beam curing can be carried out on a precursor roller 140" which has been removed from the extrusion apparatus 150, as indicated in FIG. 3, it is also possible to carry out the e-beam curing inside the extrusion apparatus.

Following the curing process, a prototype roller (such as one of rollers 140, 140' or 140") is preferably finished via a grinding and/or polishing procedure.

Subsequent to grinding and/or polishing, the outer surface of a roller can be advantageously preconditioned for use in a fusing station by forming a thin protective skin on the surface by reacting the surface with an amine-functionalized polydimethyl siloxane oil at an elevated temperature. This is preferably done by coating the surface of the roller with No. 8707 oil sold by Walker Silicone and heating the roller for about 24 hours at a temperature between about 150° C.–175° C.

As indicated, alternatively an optional, thin, overcoat can be applied to the surface, e.g., for providing a protective layer or a gloss control layer (optional protective layer or gloss control layer is shown in FIGS. 1 and 2). Thus a thin fluoropolymer coating made from a fluoro-thermoplastic formulation can be coated directly on the surface, such as for example by using the materials and methods disclosed in the Chen, et al., patents (commonly assigned U.S. Pat. Nos. 6,355,352 B1 and 6,361,829 B1). Such a coating preferably has a thickness in a range of approximately between 0.001 inch–0.004 inch.

In an alternative embodiment, the optional thin overcoat can be a layer made of a fluoroelastomer material, e.g., a VITON® material, as disclosed for example in the Chen, et al., patents (U.S. Pat. Nos. 5,464,698 and 5,595,823, assigned to Heidelberg Digital, L.L.C., Rochester, N.Y.). Such a fluoroelastomeric layer preferably has a thickness in

a range of approximately between 0.001 inch–0.004 inch (optional fluoroelastomeric overcoat not shown in FIGS. 1 and 2).

As yet another alternative, an optional, thin, layer of polytetrafluoroethylene can be spray-coated onto the surface of the roller (optional polytetrafluoroethylene overcoat not shown in FIGS. 1 and 2). Such a polytetrafluoroethylene layer preferably has a thickness in a range of approximately between 0.001 inch–0.006 inch, and more preferably in a range of approximately between 0.001 inch–0.003 inch.

However, notwithstanding an ability to provide protective overcoats, it is generally preferred not to overcoat a roller of the invention.

In the Example below, quantities of hollow expanded microballoons were blended with a commercial fluoro-thermoplastic powder and formed into plaques under combined heat and pressure. Tensile modulus was measured for each plaque using a RHEOMETRICS® RSA II Dynamic Mechanical Analyser (DMA) apparatus. No other fillers (such as strength-enhancing or thermal-conductivity-enhancing filler particles) were introduced into the formulation, nor was any catalyst or curing agent included. The object of the Example is to demonstrate that incorporation of uniformly distributed microballoons causes a significant reduction in the DMA modulus.

## EXAMPLE

### Incorporation of Microballoons into a Fluoro-thermoplastic Material

Samples were prepared in which different quantities of DE 092 particles (available from Expance, Duluth, Ga.) were blended by hand, by mixing with THV 200 powder (a fluorocarbon thermoplastic random copolymer powder obtainable from 3M® Corporation, St. Paul, Minn.). Samples 1–3, including a control sample having no added microballoon particles, were made as indicated in columns 1, 2, and 3 of Table 1.

TABLE 1

| Incorporation of DE 092 Microballoons into THV 200 |                       |                            |                          |
|----------------------------------------------------|-----------------------|----------------------------|--------------------------|
| Sample No.                                         | THV 200 Percent (w/w) | Microballoon Percent (w/w) | DMA Modulus (Megapascal) |
| 1                                                  | 100                   | 0                          | 9.05                     |
| 2                                                  | 99.5                  | 0.5                        | 7.98                     |
| 3                                                  | 99.0                  | 1.0                        | 7.39                     |

Each powder sample weighing 50 grams was poured into a square pressure mold for making a sample plaque. The mold had a base of interior dimensions 4"×4"×0.075" deep. With a powder sample in the mold, the lid of the mold was carefully placed on the powder sample, and the mold was placed into a Carver press and then heated from room temperature to a temperature between about 130° C.–140° C. This temperature is higher than the melting point of the THV 200 polymer. Pressure was then slowly applied to the mold until fully closed. While maintaining the temperature between about 130° C.–140° C., the mold was left under pressure for 10 minutes. The press was then cooled with chilled water after which the mold was removed. The sample was demolded and the DMA modulus measured at 21° C. The results are shown in column 4 of Table 1, where it may be seen that incorporation of 1.0 percent by weight (w/w) of DE 092 microballoons produced an 18% reduction of the

tensile modulus of the thermoplastic. It should be noted that according to published information available from Expance, the microballoon structural integrity should not have changed at a temperature between about 130° C.–140° C., i.e., the microballoons should not have shrunk to any significant degree. Moreover, substantially no curing of the thermoplastic took place inside the mold, and based on prior experience of the inventors with similar materials, the resulting modulus is considered close to that which would have been measured had in fact the THV 200 material been thermally crosslinked, e.g., as described in reference to FIG. 3.

It may therefore be concluded that a controlled-modulus fluoropolymer material useful for making a fusing-station roller can be prepared from dry ingredients inclusive of a fluoro-thermoplastic polymer and hollow filler particles in the form of flexible microballoons.

A method is disclosed for making a fusing-station member for use in a fusing station of an electrostatographic machine, the fusing-station member formed from a substrate and a resilient layer adhered to the substrate, the method including the steps of: mixing of ingredients so as to produce an uncured formulation, the ingredients including thermoplastic particles made of a copolymer of vinylidene fluoride, hexafluoropropylene, and tetrafluoroethylene, microsphere particles, strength-enhancing solid filler particles, thermal-conductivity-enhancing solid filler particles, and a curing catalyst, wherein the microsphere particles have a concentration in the uncured formulation in a range of approximately between 0.25%–10% by weight; forming on the substrate a curable layer of the uncured formulation, the curable layer formed with a substantially uniform thickness on the substrate; and curing of the curable layer to form a cured layer on the substrate.

The method can be applied to making the fusing-station member as a roller, either as a fuser roller or as a pressure roller, wherein the substrate is preferably a core member, the core member rigid and cylindrical. The forming is preferably carried out by extruding the uncured formulation around the core member, the uncured formulation preferably at a temperature in a range of approximately between 80° C.–200° C. during the extruding and the core member at any suitable temperature during the extruding.

Alternatively, the method can be applied to making the fusing-station member in the form of a web, with the substrate included in the web, and the forming including any suitable coating technique.

In the method, the curing of the curable layer can be a thermal curing, the thermal curing at an elevated temperature, the elevated temperature preferably in a range between approximately 150° C.–300° C., and after the thermal curing, an additional step is provided for cooling the cured layer on the substrate to room temperature. The curable layer for thermal curing can contain the microsphere particles as unexpanded microspheres, wherein the unexpanded microspheres are expanded to microballoons during the thermal curing. Alternatively, the microsphere particles in the uncured formulation can be expanded microballoons.

In an alternate curing procedure, the curing of the curable layer can be an electron-beam curing.

In summary, the invention provides a novel fusing-station member inclusive of a durable, tough, elastically deformable layer incorporating hollow flexible filler particles, wherein the hollow flexible filler particles provide a controlled modulus. The elastically deformable layer is preferably a single layer on a substrate, the substrate preferably a core member of a fuser roller or a pressure roller. The elastically

19

deformable layer is made from a dry formulation inclusive of: a fluoro-thermoplastic polymer powder; microspheres in the form of unexpanded microspheres or expanded microballoons; and solid filler particles including strength-enhancing filler particles and thermal-conductivity-enhancing filler particles. The dry formulation can be thermally cured or electron-beam cured. Preferably, the dry formulation is thermally cured and further includes a curing catalyst, preferably a peroxide catalyst for thermal curing at a temperature in a range of approximately between 150° C.–200° C. Alternatively, the curing catalyst can be a bisphenol residue for thermal curing at a temperature in a range of approximately between 250° C.–300° C.

The invention has been described in detail with particular reference to certain preferred embodiments thereof, but it will be understood that variations and modifications can be effected within the spirit and scope of the invention.

What is claimed is:

1. A fusing-station roller for use in a fusing station of an electrostatographic machine, said fusing-station roller elastically deformable, said fusing-station roller comprising: a core member, said core member rigid and having a cylindrical outer surface; a resilient layer, said resilient layer formed on said core member; wherein said resilient layer is a fluoropolymer material, said fluoropolymer material made from an uncured formulation by a curing; wherein said uncured formulation includes a fluoro-thermoplastic polymer, said fluoro-thermoplastic polymer comprising a copolymer, said copolymer made of monomers of vinylidene fluoride ( $\text{CH}_2\text{CF}_2$ ), hexafluoropropylene ( $\text{CF}_2\text{CF}(\text{CF}_3)$ ), and tetrafluoroethylene ( $\text{CF}_2\text{CF}_2$ ), said copolymer having a composition of:



wherein,

x is from 1 to 50 mole percent,

y is from 9 to 59 mole percent,

z is from 40 to 90 mole percent,

x+y+z equals 100 mole percent;

wherein said uncured formulation includes microsphere particles, said microsphere particles having flexible walls;

wherein said microsphere particles have a predetermined weight percentage in said uncured formulation; and wherein in addition to said microsphere particles, said uncured formulation includes solid filler particles.

2. The fusing-station roller of claim 1, wherein a type of solid filler particles includes strength-enhancing filler particles.

3. The fusing-station roller of claim 2, wherein said strength-enhancing filler particles are members of a group including particles of silica, zirconium oxide, boron nitride, silicon carbide, carbon black, and tungsten carbide.

4. The fusing-station roller of claim 2, wherein said strength-enhancing filler particles have a concentration in said uncured formulation in a range of approximately between 2.5%–10% by weight.

5. The fusing-station roller of claim 1, wherein a type of solid filler particles includes thermal-conductivity-enhancing filler particles.

6. The fusing-station roller of claim 5, wherein said thermal-conductivity-enhancing filler particles are selected from a group including particles of aluminum oxide, iron

20

oxide, copper oxide, calcium oxide, magnesium oxide, nickel oxide, tin oxide, zinc oxide, graphite, carbon black, and mixtures thereof.

7. The fusing-station roller of claim 5, wherein said thermal-conductivity-enhancing filler particles have a concentration in said uncured formulation in a range of approximately between 10%–40% by weight.

8. The fusing-station roller of claim 5, wherein said thermal-conductivity-enhancing filler particles have a concentration in said uncured formulation in a range of approximately between 40%–70% by weight.

9. The fusing-station roller of claim 1, wherein said microsphere particles are hollow microballoons, said hollow microballoons having at least one distinguishable size.

10. The fusing-station roller of claim 9, wherein said hollow microballoons have diameters of up to approximately 120  $\mu\text{m}$ .

11. The fusing-station roller of claim 1, wherein said microsphere particles are unexpanded microspheres, said unexpanded microspheres being expanded to microballoons during said curing, said curing being carried out at an elevated temperature.

12. The fusing-station roller of claim 11, wherein said microballoons are hollow, flexible, and have at least one distinguishable size.

13. The fusing-station roller of claim 1, wherein said predetermined microsphere concentration is in a range of approximately between 0.25%–10% by weight in said uncured formulation.

14. The fusing-station roller of claim 13, wherein said predetermined microsphere concentration is in a range of approximately between 0.5%–4% by weight in said uncured formulation.

15. The fusing-station roller of claim 1, wherein said curing is a thermal curing, said thermal curing carried out at an elevated temperature.

16. The fusing-station roller of claim 15, wherein said elevated temperature is in a range of approximately between 150° C.–200° C.

17. The fusing-station roller of claim 15, wherein said elevated temperature is in a range of approximately between 250° C.–300° C.

18. The fusing-station roller of claim 1, wherein said curing of said uncured formulation is an electron-beam curing.

19. The fusing-station roller of claim 1, wherein said flexible walls of said microsphere particles include a polymeric material, said polymeric material polymerized from monomers selected from the following group of monomers: acrylonitrile, methacrylonitrile, acrylate, methacrylate, vinylidene chloride, and combinations thereof.

20. The fusing-station roller of claim 1, wherein said flexible walls of said microsphere particles include finely divided particles selected from a group including inorganic particles and organic polymeric particles.

21. The fusing-station roller of claim 1, wherein a thickness of said resilient layer has an upper limit of approximately 0.1 inch.

22. The fusing-station roller of claim 21, wherein a thickness of said resilient layer is in a range of approximately between 0.005 inch–0.02 inch.

23. The fusing-station roller of claim 1, wherein said fusing-station roller is a fuser roller, said fuser roller internally heated.

24. The fuser roller of claim 23, wherein said thermal conductivity of said resilient layer is in a range of approximately between 0.08 BTU/hr/ft<sup>2</sup> F.–0.7 BTU/hr/ft<sup>2</sup> F.

**21**

**25.** The fuser roller of claim **24**, wherein said thermal conductivity of said resilient layer is in a range of approximately between 0.2 BTU/hr/ft/<sup>o</sup> F.–0.5 BTU/hr/ft/<sup>o</sup> F.

**26.** The fusing-station roller of claim **1**, wherein said fusing-station roller is a fuser roller, said fuser roller being externally heated.

**27.** The fuser roller of claim **26**, wherein said thermal conductivity of said resilient layer has an upper limit of approximately 0.4 BTU/hr/ft/<sup>o</sup> F.

**28.** The fuser roller of claim **27**, wherein said thermal conductivity of said resilient layer is in a range of approximately between 0.1 BTU/hr/ft/<sup>o</sup> F.–0.35 BTU/hr/ft/<sup>o</sup> F.

**29.** The fusing-station roller of claim **1**, wherein a Shore A durometer of said resilient layer is in a range of approximately between 50–80.

**30.** The fusing-station roller of claim **29**, wherein a Shore A durometer of said resilient layer is in a range of approximately between 60–70.

**22**

**31.** The fusing-station roller of claim **1**, wherein said fusing-station roller is a pressure roller.

**32.** The pressure roller of claim **31**, wherein a thermal conductivity of said resilient layer is in a range of approximately between 0.1 BTU/hr/ft/<sup>o</sup> F.–0.2 BTU/hr/ft/<sup>o</sup> F.

**33.** The fusing-station roller of claim **1**, wherein said solid filler particles have a mean diameter in a range of approximately between 0.1  $\mu$ m–100  $\mu$ m.

**34.** The fusing-station roller of claim **34**, wherein said solid filler particles have a mean diameter in a range of approximately between 0.5  $\mu$ m–40  $\mu$ m.

**35.** The fusing-station roller of claim **1**, wherein said fluoro-thermoplastic polymer in said uncured formulation is in a form of particles, said particles having diameters in a range of approximately between 0.01 mm–1 mm.

\* \* \* \* \*